

May 19, 1953

2,639,257

A. SZEGVARI ET AL  
PROCESS FOR MAKING TRANSDUCER DEVICES  
HAVING BONDED ELEMENTS  
Filed May 3, 1950



FIG. 1



FIG. 2

INVENTOR.  
ANDREW SZEGVARI  
CHARLES K. GRAVLEY  
BY

*Harries A. Mamula Jr.*

ATTORNEY

## UNITED STATES PATENT OFFICE

2,639,257

PROCESS FOR MAKING TRANSDUCER  
DEVICES HAVING BONDED ELEMENTS

Andrew Szegvari, Akron, and Charles K. Gravley, Lakewood, Ohio, assignors to The Brush Development Company, Cleveland, Ohio, a corporation of Ohio

Application May 3, 1950, Serial No. 159,746

18 Claims. (Cl. 154—140)

1

This invention relates to an improved process for making a transducer device, and, more particularly, to a process for making such a device having an electromechanically sensitive or piezoelectric element one surface of which is secured to another similarly shaped surface.

One type of device which may be produced by the improved process of the invention may be called an expander piezoelectric transducer. This type of device includes an electromechanically sensitive element which may be a bar cut from a single crystal having piezoelectric properties. The bar is electrodeed so that alternating electrical energy applied to the electrodes is associated with alternating lengthwise mechanical expansions and contractions of the bar. Likewise, mechanical forces applied so as to cause lengthwise expansion and contraction cause the generation of electrical energy at the electrodes. One end surface of the bar is flat and is secured to another similarly shaped surface such as a flat base surface. Mechanical or acoustical energy then may be applied or utilized at the other end of the bar.

The process of the invention also may be used to secure together the several piezoelectric elements or plates of a sandwich type of transducer in which two or more piezoelectric plates are affixed face to face to provide a flexural motion. A device which may be called a series-connected bender sandwich transducer is illustrated in Figs. 4 and 5 of the patent to Charles B. Sawyer, Reissue No. 20,213. Two crystal plates are secured together and the exposed outer major surfaces electrodeed. Applying a voltage across these electrodes causes one plate to tend to expand in one direction and the other plate to tend to contract in the same direction along the major surfaces of the plates, giving a resultant over-all bending motion. A flexural device also may be made by securing together two piezoelectric plates which tend to have face shear distortions in opposite senses when the voltage is applied, giving a resultant twisting motion.

In the electromechanical transducer devices of the types mentioned, it is important that the surface or surfaces of the piezoelectric element or elements be well secured. If the surfaces should break apart, the transducer device cannot function until repaired. If the bond between the surfaces should be soft or unduly resilient, some of the motion representing the mechanical energy which it is desired to apply to or take from the device will be lost. A failure of adherence over part but not all of the surfaces to be bonded

also may cause undesirable changes in the performance of the transducer.

Various methods and materials have been tried for bonding or affixing the electromechanically sensitive elements to base surfaces or to other matching elements, some with a rather high degree of success. For example, two elements cut from single crystals of Rochelle salt may be affixed to each other using small amounts of Rochelle salt itself dissolved in its water of crystallization by heating. However, this method has several disadvantages, including poor dimensional stability in the presence of moisture and poor insulation resistance. Various other cements, including some using polymerizable materials, have been tried for securing crystal surfaces. Many of these cements harden or set with the elimination of a volatile solvent, and poor results are obtained frequently when the solvent has to escape from the middle of a rather large sandwich structure. Long periods of time or excessively high temperatures are required to obtain bonding with some of these materials. Uniformly strong bonding has been very difficult to achieve. Thus it may be said that an ideal answer to this problem has not been found.

It is an object of this invention, therefore, to provide a new and improved process for making a transducer device having an electromechanically sensitive element, one surface of which is secured to another similarly shaped surface, in which one or more of the disadvantages of the prior art processes is avoided.

It is another object of this invention to provide a new and improved process for making such a transducer device in which the cementing material is non-aqueous and free of volatile solvent.

It is a further object of the invention to provide a new and improved process for making such a transducer device which may be carried out in short periods of time at temperatures well under the boiling point of water.

It is still another object of the invention to provide a new and improved process for making such a transducer device by means of which there is obtained easily and inexpensively a uniform and very strong bond.

In accordance with the invention, the process for making a transducer device having an electromechanically sensitive element, one surface of which is secured to another similarly shaped surface, comprises applying to at least one of these two surfaces a bonding material, which is partially polymerized to enable further rapid polymerization for bonding purposes at temperatures

2

not highly elevated, and which is in a state of molecular dispersion in a quantity of a polymerizable liquid solvent material to increase the liquidity of the bonding material and permit a satisfactory bonding contact with elemental areas of the aforesaid surfaces in spite of the substantially large average molecular size of the partially polymerized bonding material. The process further comprises placing the two surfaces one against the other with the introduction there-between of a catalyst to effect a polymerization reaction involving simultaneously the partially polymerized bonding material and the polymerizable solvent material at a temperature under 90° C. without evolution of any volatile material, thereby effecting strong adhesion of the two surfaces.

For a better understanding of the present invention, together with other and further objects thereof, reference is had to the following description taken in connection with the accompanying drawing, and its scope will be pointed out in the appended claims.

In the drawing,

Fig. 1 is a perspective view partially cut away, of an expander transducer device assembled in accordance with the process of the invention; and

Fig. 2 is a perspective view of a series-connected bender transducer made in accordance with the invention.

Referring to Fig. 1 of the drawing, there is shown a transducer assembly including a base surface 11 on which rests a block or bar 12 of piezoelectric material. The bar 12 rests on the base 11 at a surface portion 13 of the base 11, visible where a corner portion of the bar 12 has been cut away. The bar 12 is provided with electrodes 14 and 16 on individual opposed surfaces of the bar. The bar 12 may be cut from a single crystal of Rochelle salt in a well known manner so that distortion of the bar, involving a vertical movement of the upper surface of the bar, as indicated by the double arrow, is associated with the application or appearance of an electrical voltage or charge at the electrodes 14 and 16. The length dimension of the bar is assumed to be the vertical dimension in Fig. 1, but it is understood that this vertical dimension of the bar may be considerably smaller and may even be the thickness dimension of the bar. The bar 12 resting on the surface 11 may be placed in a body of liquid such as oil, in which case movements of the upper surface of the bar are communicated to the liquid and may cause the generation of acoustical elastic wave energy in the liquid. Many forms of such electroacoustical transducers are known to the art. For example, a number of other bars, not shown, similar to the bar 12 may be placed on the base surface 11 side by side with the bar 12 and their respective electrodes connected to the same source of electrical energy. The top surfaces of such a plurality of piezoelectric bars may be connected to a relatively large diaphragm, not shown, covering all of the bars to obtain the desired acoustical coupling to a fluid or liquid medium.

In such devices it is necessary that the lower surface of the bar 12 and of any similarly arranged bars in the electroacoustical transducer be well secured to the base 11 at the surface or surfaces 13 of contact. Not only must the assembly remain secure during transportation and in use, even if the base surface 11 is turned on its side or is turned over so as to face vertically

downward, but also the bond must be secure against acoustical vibrations in the liquid, to which the free end surface of the bar is coupled and which may exert forces on the bar tending to pull it away from the base 11. The process of the invention for making a transducer device such, for example, as the device in which the electromechanically sensitive element 12 is secured to the surface 13 will be described in detail hereinbelow.

Referring now to Fig. 2 of the drawing, there is shown a series-connected bending-sensitive transducer assembly of the sandwich type including a base 21. The transducer also includes two electromechanically sensitive elements 22 and 23. A major surface of one of these elements is placed against a major surface of the other element, and one end portion of the resulting assembly is fastened within a depression machined in the base 21. This fastening may be accomplished by clamping, by the insertion of shims around the end portion of the electromechanically sensitive assembly, or with the use of the cementing procedure specified in accordance with the present invention as described in detail hereinbelow. The exposed or outer major surfaces of the elements 22 and 23 are provided with respective electrodes 24 and 26, a portion of the latter being visible in Fig. 2 where the electrode 24 and the elements 22 and 23 have been cut away. The free end portion of the composite element assembly is provided with a channel member 27 clamped securely thereover. To the channel member is fastened, as by welding, a rod 28.

The electrodes 24 and 26 may be connected to respective electrical terminals, not shown. Any voltage appearing across such electrodes is applied in series across the elements 22 and 23. For this reason the composite sandwich element may be called a series-connected sandwich type transducer. The elements 22 and 23 may be plates cut from single crystals of a piezoelectric substance such as Rochelle salt or ammonium dihydrogen phosphate. The two plates may be identical, but during assembly the plates are turned so that the thickness directions of the two plates are oriented oppositely with respect to the piezoelectric axes of the crystalline substance. Accordingly one plate tends to expand while the other contracts, so that an electric field across the plates is associated with piezoelectric deformations of the regions near the two adjacent surfaces in opposite senses, these deformations in turn being associated with flexural movements of the composite element, specifically bending movements of vertical lines in the composite element as seen in Fig. 2. When the composite element bends, the rod 28 moves axially, as indicated by the double arrow. Likewise forces applied axially to the rod 28 are transmitted through the channel 27 to cause over-all bending movements of the composite element, one element being elongated while the other element is shortened. This is the same type of transducer device illustrated in Figs. 4 and 5 of the Sawyer reissue patent, referred to hereinabove.

In sandwich type transducer devices such as that shown in Fig. 2, it frequently is desirable to electrode the inner surfaces of each of the plates 22 and 23 before placing them together. This permits a parallel rather than a series connection of the two elements. Moreover, very thin electrodes of finely divided conductive particles may be applied to make intimate contact with the surfaces, so that when the two electrode sur-

faces are placed in contact with each other there are no spaces between the crystalline surfaces across which voltage drops might develop due to the relatively low dielectric constants of the cementing materials. In such cases it is customary to leave substantial unelectroded margins around the edges of the opposed surfaces. When these partially electroded surfaces are placed in proximity to each other, a particularly strong bond may be achieved in accordance with the present invention between the unelectroded marginal surface portions of the two single-crystalline plates of piezoelectric material. The bonding process described hereinbelow also produces a very good bond between electroded portions of the two crystal surfaces.

The process in accordance with the invention for making a transducer device, such as the device in which the electromechanically sensitive elements 22 and 23 of Fig. 2 are secured to each other, now will be described.

The process for making a transducer device having an electromechanically sensitive element, such as the element 12 of Fig. 1 or each of the elements 22 and 23 of Fig. 2, one surface of which is secured to another similarly shaped surface, comprises applying to at least one of these two surfaces a bonding material which is partially polymerized to enable further rapid polymerization for bonding purposes at temperatures not highly elevated. If a monomeric compound such as the monoester of a dicarboxylic acid and a glycol were used as the bonding material, or if a slightly polymerized material such as the dimer of such a monoester were used, the polymerization needed to achieve a satisfactory bond is so extensive that inconveniently large periods of time, or temperatures so elevated as to be damaging to piezoelectric crystals, or both, would be required to make the bonding material set or harden. However, the partially polymerized materials which conveniently may be further polymerized have lost to an noticeable extent their ability as liquids to spread over the surfaces to be bonded and to penetrate to all minute portions of such surfaces. Accordingly the partially polymerized bonding material is applied to at least one of these surfaces in a state of molecular dispersion in a quantity of a polymerizable liquid solvent material to increase the liquidity of the bonding material and permit a satisfactory bonding contact with elemental areas of the surfaces in spite of the substantially large average molecular size of the partially polymerized bonding material. The process, broadly expressed, then comprises placing the two surfaces so treated one against the other with the introduction therebetween of a catalyst to effect a polymerization reaction involving most or all of the material which had been applied, thus effecting the bond, as described and exemplified in detail hereinbelow. It would be permissible to include between the surfaces to be secured together some inert substance, provided the setting process can be carried out at a temperature under 90° C. without evolution of any volatile material. However, it is preferred to use only active or polymerizable substances in the bonding material, so that when the surfaces are placed together in the presence of the catalyst a polymerization reaction is effected involving directly all materials used in the bonding operation.

As a bonding material it is preferred to use an essentially linear olefinic polyester. A suitable polyester is a polyester of a dicarboxylic acid

and a glycol. The partially polymerized state of the polyester bonding material preferably provides molecular weights of the order of 2000, but in any case the polyesters should have a molecular weight less than about 5000. The condensation polymerization of the esters of dicarboxylic acids and dihydric alcohols to form linear polyesters is well known. This polymerization reaction can be made to proceed smoothly in the presence of catalysts conventionally used for this purpose, particularly when the acid and alcohol are present in fairly pure forms and in stoichiometrically equivalent amounts. An identical polyester may be obtained when the corresponding monomeric ester or monoester, which is both an acid ester and an ester-alcohol, is formed by reacting the glycol with the anhydride of the particular dicarboxylic acid. Accordingly the preferred process of the present invention may be carried out using polyesters obtained from such anhydrides or in any other suitable manner, even though the original reaction forming the monoester cannot be designated strictly as a condensation or even an esterification reaction. The expression, "a polyester of a dicarboxylic acid and a glycol," as used in this specification and in the appended claims, is intended to include polyesters having the specified composition whether or not actually formed by the esterification of a dicarboxylic acid and a glycol under polymerizing conditions.

The monoester of a given dicarboxylic acid and a given glycol can be formed. For example, equimolecular amounts of maleic acid



and diethylene glycol,  $\text{CH}_2\text{OH} \cdot \text{CH}_2 \cdot \text{O} \cdot \text{CH}_2 \cdot \text{CH}_2\text{OH}$ , would form a monoester, diethylene glycol maleate, having a molecular weight of 204, having a hydroxy group at one end of the molecule and a carboxy group at the other end, and having one olefinic linkage in the molecular chain containing eight carbon atoms and the oxygen atom from the diethylene glycol. However, with or without some catalytic action or the aid of an accelerator, the polymerization of this monoester usually proceeds to some degree, and so is carried out at least to a significant extent before the material is used in the process of the present invention. Thus polyesters are formed having molecular weights which presumably are approximate multiples of the molecular weight of the monoester. Accordingly, it is desirable to carry out a substantial partial polymerization of the esterification product to obtain a partially polymerized polyester having a moderate molecular weight, as mentioned hereinabove. The polyester thus formed may be very viscous, and its classification either as a liquid or as a solid may not be obvious. Such polyesters formed from polybasic acids or anhydrides and polyhydric alcohols by the condensation polymerization of a monoester are known as alkyd resins. Viscous, partially polymerized resins of this type may be used directly as bonding agents by causing further polymerization, but, as mentioned above, the local mobility and the liquidity of the material are so low that a good bond is difficult to achieve.

Therefore, before the partially polymerized bonding material is used in making the transducer device in accordance with the invention, it is placed in a state of molecular dispersion in a quantity of a polymerizable liquid solvent material, preferably a polymerizable liquid aromatic

compound with an olefinic side chain. The individual molecules of the partially polymerized material are dispersed in the liquid without chemical breakdown of the molecules. A quantity of essentially monomeric styrene



is admirably suited for this purpose, but other compounds of this type, such as diallyl phthalate,  $\text{O}-\text{C}_8\text{H}_4(\text{CO.O.CH}_2\text{CH}:\text{CH}_2)_2$ , also are suitable.

When the polyester bonding material is in solution in a quantity of styrene, as just described, the resulting material not only has high local mobility and in general rather low viscosity but also can be polymerized quite readily and completely at temperatures not at all highly elevated. This high liquidity permits easy spreading of the material to all portions of the surfaces to be bonded, and it has been observed that these polyesters dissolved in styrene tend to wet the surfaces of the usual electromechanically sensitive elements. Once having spread over and covered these surfaces, the local mobility of the material tends to insure active contact of the solution with each submicroscopic portion of the surface of the element. The effectiveness of this active contact seems to be particularly great when the surface covered is that of a body of a substance which is polar, so that especially good bonding may be obtained when at least one of the two surfaces to be secured together is cut from a single crystal of a polar compound.

The phrase "a dicarboxylic acid" is used herein in the collective sense, and such an acid may contain in admixture or in solution more than one dicarboxylic acid. Likewise, more than one glycol might be used. In such cases presumably the dicarboxylic acids and the glycols enter the linear polymeric chain in the approximate relative proportions of their original molecular ratios. However, it is generally important that, considering all dicarboxylic acid substances present on the one hand and all glycol substances present on the other hand, these substances be present originally in stoichiometrically equivalent ratios. Thus, when the polyester is of the type formed by the condensation of a single dibasic acid and a single glycol, the polyester may be produced from equimolecular amounts of the particular acid and the particular glycol.

The polyester used advantageously is at least partially olefinic. In other words, at least some of the monoester units making up the polyester molecule advantageously should be olefinic. This can be accomplished by using either a dicarboxylic acid, or a glycol, or both, which contains an olefinic acid or glycol, as the case may be.

In a preferred form of the process of the invention, the dicarboxylic acid contains at least substantial portions of an olefinic dicarboxylic acid to provide in the polyester at least a substantial number of olefinic monoester components, making the corresponding polyester at least partially olefinic. Accordingly the dicarboxylic acid may contain at least substantial portions of maleic acid. The dicarboxylic acid may consist solely of an olefinic dicarboxylic acid to make the polyester produced by reaction with a glycol under polymerizing conditions an olefinic polyester. When the dicarboxylic acid contains substantial portions of an olefinic dicarboxylic acid, it may also contain a saturated dicarboxylic acid, such as sebacic acid,  $\text{COOH}(\text{CH}_2)_8\text{COOH}$ . Thus the dicarboxylic acid constituents of the

polyester may contain or consist of sebacic acid and substantial portions of maleic acid, or the olefinic polyester may be the polyester of a single dicarboxylic acid, preferably maleic acid, and a glycol.

5 A variety of glycols is available for the formation of the polyester used in connection with the invention. The simpler glycols are preferred, and excellent results have been obtained with the olefinic polyester of ethylene glycol,



15 and a dicarboxylic acid containing substantial portions of maleic acid. Diethylene glycol may be used, and one olefinic polyester which has given particularly good results is the polyester of maleic acid and diethylene glycol, the mono-ester of which is mentioned hereinabove. It will

20 be understood that the particular polyester just referred to does not contain in its molecules any appreciable acidic or alcoholic components other than those which may be derived by the polyesterification mechanism from the specified di-  
25 basic acid and glycol; however, it will be clear that identical polyesters, described and defined by the same names, may be formed with anhydrides instead of acids, for example, by the use of maleic anhydride,



30 35 instead of maleic acid.

After the olefinic polyester has been dissolved in the styrene, it is applied to at least one of the two surfaces to be secured together.

In a preferred embodiment of the invention, 40 100 parts by weight of the product formed by the condensation of maleic acid and diethylene glycol are dissolved in 30 parts of nominally monomeric styrene by stirring vigorously until a homogeneous solution is obtained. In this form the solution has a shelf life of several months. The 45 solution is applied to one of the two surfaces, while a catalyst is applied to the other of the surfaces, so that when the two surfaces subsequently are placed one against the other the catalyst automatically is introduced therebetween and immediately starts to bring about the desired polymerization reaction involving simultaneously the partially polymerized polyester bonding material and the polymerizable solvent styrene material, thereby effecting strong adhesion of the two surfaces. Four parts of a peroxide catalyst in the form of benzoyl peroxide,  $(\text{C}_6\text{H}_5\text{CO})_2\text{O}_2$ , may be used with the maleate-styrene solution specified above. This peroxide 50 material conveniently is dissolved in a non-aqueous solvent and applied in liquid form, for example as a 5% solution in benzene. The liquid catalyst solution is allowed to dry before the surface to which it has been applied is pressed against the surface to which the polyester-styrene solution has been applied.

55 Other catalysts, mostly of the peroxide type, suitable for use in the present process are well known in the art. For example, lauroyl peroxide,  $(\text{CH}_3(\text{CH}_2)_{10}\text{CO})_2\text{O}_2$ , or a cyclic organic peroxide may be used, preferably in combinations with an accelerator such as a cobalt salt of naphthenic acids. The polymerization reaction proceeds in a period of time of the order of one hour, and frequently less than half an hour, to provide a

well set bond of the plastic material, and this setting occurs in the short period of time at a temperature under 90° C. Using many of the specific materials mentioned hereinabove, the polymerization proceeds in the neighborhood of room temperature to substantial completion in a short period of time, so that the process of the invention is particularly useful when materials are involved which should not be subjected to higher temperatures.

In another preferred embodiment of the invention, 100 parts by weight of a partially polymerized polyester material are dissolved in 35 parts of styrene, and about 0.1 part of cobalt naphthenate is added to the liquid. This liquid has a long shelf life. Within about half an hour before the time of applying the bonding material, 0.8 part of lauroyl peroxide powder is added to the liquid as a catalyst. The resulting solution is applied promptly to both surfaces to be secured together, so that the catalyst is introduced between the surfaces at the time of application along with the bonding material itself. The catalyzed material has a setting time of about three hours at 50° C., during which time the two surfaces are maintained pressed together. This procedure, using the specified materials, has been particularly successful. The polyester material used conveniently is made up of 25 parts of "Paraplex AP48" and 75 parts of "Paraplex AP45," these being products obtainable from the Rohm & Haas Company, Philadelphia. These products are polyesters which are essentially the condensation products of sebacic acid, maleic acid, and ethylene glycol, the "AP48" material having proportionately less of the olefinic maleic acid than the "AP45" material.

While an understanding of the mechanism of the polymerization reaction is not a part of the present invention, it will appear that all the cementing materials used with the possible exception of the catalyst itself are polymerizable and should take an active part in the cementing process. This occurs without evolution of any volatile material, since no such material need be present between the two surfaces when they are placed together. It is believed that the styrene serves to provide a substantial number of cross linkages with linear polyester chains by virtue of the double bonds in the unsaturated polyester and in the styrene itself. Thus the catalyst acts to effect a polymerization and cross-linking reaction. A tensile strength greater than that of the piezoelectric crystals themselves may be obtained, and the bonding material is quite resistant to moisture and non-aqueous solvents. In the usual transducer configurations the exothermic nature of the polymerization reaction causes only a small temperature rise. This polymerization tends to be inhibited by air, making it possible to wipe off surplus cement after the joint has set.

While there have been described what at present are considered to be the preferred embodiments of this invention, it will be obvious to those skilled in the art that various changes and modifications may be made therein without departing from the invention. It is aimed, therefore, in the appended claims to cover all such changes and modifications which fall within the true spirit and scope of the invention.

What is claimed is:

1. The process for making a transducer device having an electromechanically sensitive element one surface of which is secured to another simi-

larly shaped surface comprising: applying to at least one of said two surfaces a bonding material, which is partially polymerized to enable further rapid polymerization for bonding purposes at temperatures not highly elevated, and which is in a state of molecular dispersion in a quantity of a polymerizable liquid solvent material to increase the liquidity of said bonding material and permit a satisfactory bonding contact with elemental areas of said surfaces in spite of the substantially large average molecular size of said partially polymerized bonding material; and placing said two surfaces one against the other with the introduction therebetween of a catalyst to effect a polymerization reaction involving simultaneously said partially polymerized bonding material and said polymerizable solvent material at a temperature under 90° C. without evolution of any volatile material, thereby effecting strong adhesion of said two surfaces.

2. The process for making a transducer device having an electromechanically sensitive element one surface of which is secured to another similarly shaped surface comprising: applying to at least one of said two surfaces a polyester, which is partially polymerized to enable further rapid polymerization for bonding purposes at temperatures not highly elevated, and which is in a state of molecular dispersion in a quantity of a polymerizable liquid solvent material to increase the liquidity of said polyester and permit a satisfactory bonding contact with elemental areas of said surfaces in spite of the substantially large average molecular size of said partially polymerized polyester; and placing said two surfaces one against the other with the introduction therebetween of a catalyst to effect a polymerization reaction involving simultaneously said partially polymerized polyester and said polymerizable solvent material at a temperature under 90° C. without evolution of any volatile material, thereby effecting strong adhesion of said two surfaces.

3. The process for making a transducer device having an electromechanically sensitive element one surface of which is secured to another similarly shaped surface comprising: applying to at least one of said two surfaces an essentially linear polyester, which is partially polymerized to enable further rapid polymerization for bonding purposes at temperatures not highly elevated, and which is in a state of molecular dispersion in a quantity of a polymerizable liquid solvent material to increase the liquidity of said polyester and permit a satisfactory bonding contact with elemental areas of said surfaces in spite of the substantially large average molecular size of said partially polymerized polyester; and placing said two surfaces one against the other with the introduction therebetween of a catalyst to effect a polymerization reaction involving simultaneously said partially polymerized polyester and said polymerizable solvent material at a temperature under 90° C. without evolution of any volatile material, thereby effecting strong adhesion of said two surfaces.

4. The process for making a transducer device having an electromechanically sensitive element one surface of which is secured to another similarly shaped surface comprising: applying to at least one of said two surfaces an essentially linear olefinic polyester, which is partially polymerized to enable further rapid polymerization for bonding purposes at temperatures not highly elevated, and which is in a state of molecular dispersion in

a quantity of a polymerizable liquid aromatic compound with an olefinic side chain to increase the liquidity of said polyester and permit a satisfactory bonding contact with elemental areas of said surfaces in spite of the substantially large average molecular size of said partially polymerized polyester; and placing said two surfaces one against the other with the introduction therebetween of a catalyst to effect a polymerization and cross-linking reaction involving simultaneously said partially polymerized polyester and said polymerizable aromatic compound at a temperature under 90° C. without evolution of any volatile material, thereby effecting strong adhesion of said two surfaces.

5. The process for making a transducer device having an electromechanically sensitive element one surface of which is secured to another similarly shaped surface comprising: applying to at least one of said two surfaces a polyester of a dicarboxylic acid and a glycol, at least some of whose monoester units are olefinic, which has a molecular weight less than about 5000, and which is in solution in a quantity of a polymerizable liquid aromatic compound with an olefinic side chain; and placing said two surfaces one against the other with the introduction therebetween of a catalyst to effect a polymerization and cross-linking reaction involving said polyester and said aromatic compound at a temperature under 90° C. without evolution of any volatile material, thereby effecting strong adhesion of said two surfaces.

6. The process for making a transducer device having an electromechanically sensitive element one surface of which is secured to another similarly shaped surface comprising: applying to at least one of said two surfaces a polyester of a dicarboxylic acid and a glycol, at least some of whose monoester units are olefinic, which has a molecular weight less than about 5000, and which is in solution in a quantity of styrene; and placing said two surfaces one against the other with the introduction therebetween of a peroxide catalyst to effect a polymerization reaction involving said polyester and said styrene at a temperature under 90° C. without evolution of any volatile material, thereby effecting strong adhesion of said two surfaces.

7. The process for making a transducer device having an electromechanically sensitive element one surface of which is secured to another similarly shaped surface comprising: applying to at least one of said two surfaces an olefinic alkyd resin which has a molecular weight less than about 5000 and which is in solution in a quantity of styrene; and placing said two surfaces one against the other with introduction therebetween of a peroxide catalyst to effect a polymerization reaction involving said resin and said styrene at a temperature under 90° C. without evolution of any volatile material, thereby effecting strong adhesion of said two surfaces.

8. The process for making a transducer device having an electromechanically sensitive element one surface of which is secured to another similarly shaped surface comprising: applying to at least one of said two surfaces a polyester of a dicarboxylic acid and a glycol, said dicarboxylic acid containing at least substantial portions of an olefinic dicarboxylic acid to provide in said polyester at least a substantial number of olefinic monoester components, making said polyester at least partially olefinic, and said polyester hav-

ing a molecular weight less than about 5000 and being in solution in a quantity of styrene; and placing said two surfaces one against the other with the introduction therebetween of a peroxide catalyst to effect a polymerization reaction involving said polyester and said styrene at a temperature under 90° C. without evolution of any volatile material, thereby effecting strong adhesion of said two surfaces.

10. The process for making a transducer device having an electromechanically sensitive element one surface of which is secured to another similarly shaped surface comprising: applying to at least one of said two surfaces a polyester of a dicarboxylic acid and a glycol, said dicarboxylic acid containing a saturated dicarboxylic acid and substantial portions of an olefinic dicarboxylic acid to provide in said polyester a substantial number of olefinic monoester components, making said polyester partially olefinic, and said polyester having a molecular weight less than about 5000 and being in solution in a quantity of styrene; and placing said two surfaces one against the other with the introduction therebetween of a peroxide catalyst to effect a polymerization reaction involving said polyester and said styrene at a temperature under 90° C. without evolution of any volatile material, thereby effecting strong adhesion of said two surfaces.

15. The process for making a transducer device having an electromechanically sensitive element one surface of which is secured to another similarly shaped surface comprising: applying to at least one of said two surfaces a polyester of a dicarboxylic acid and a glycol, said dicarboxylic acid containing sebacic acid and substantial portions of an olefinic dicarboxylic acid to provide in said polyester a substantial number of olefinic monoester components, making said polyester partially olefinic, and said polyester having a molecular weight less than about 5000 and being in solution in a quantity of styrene; and placing said two surfaces one against the other with the introduction therebetween of a peroxide catalyst to effect a polymerization reaction involving said polyester and said styrene at a temperature under 90° C. without evolution of any volatile material, thereby effecting strong adhesion of said two surfaces.

20. The process for making a transducer device having an electromechanically sensitive element one surface of which is secured to another similarly shaped surface comprising: applying to at least one of said two surfaces a polyester of a dicarboxylic acid and a glycol, said dicarboxylic acid containing at least substantial portions of maleic acid to provide in said polyester at least a substantial number of olefinic monoester components, making said polyester at least partially olefinic, and said polyester having a molecular weight of less than about 5000 and being in solution in a quantity of styrene; and placing said two surfaces one against the other with the introduction therebetween of a peroxide catalyst to effect a polymerization reaction involving said polyester and said styrene at a temperature under 90° C. without evolution of any volatile material, thereby effecting strong adhesion of said two surfaces.

25. The process for making a transducer device having an electromechanically sensitive element one surface of which is secured to another similarly shaped surface comprising: applying to at least one of said two surfaces a polyester of a

13

dicarboxylic acid and a glycol, said dicarboxylic acid consisting of sebamic acid and substantial portions of maleic acid, to provide in said polyester a substantial number of olefinic monoester components, making said polyester partially olefinic, and said polyester having a molecular weight less than about 5000 and being in solution in a quantity of styrene; and placing said two surfaces one against the other with the introduction therebetween of a peroxide catalyst to effect a polymerization reaction involving said polyester and said styrene at a temperature under 90° C. without evolution of any volatile material, thereby effecting strong adhesion of said two surfaces.

13. The process for making a transducer device having an electromechanically sensitive element one surface of which is secured to another similarly shaped surface comprising: applying to at least one of said two surfaces an olefinic polyester of ethylene glycol and a dicarboxylic acid containing substantial portions of maleic acid, said polyester having a molecular weight less than about 5000 and being in solution in a quantity of styrene; and placing said two surfaces one against the other with the introduction therebetween of a peroxide catalyst to effect a polymerization reaction involving said polyester and said styrene at a temperature under 90° C. without evolution of any volatile material, thereby effecting strong adhesion of said two surfaces.

14. The process for making a transducer device having an electromechanically sensitive element one surface of which is secured to another similarly shaped surface comprising: applying to at least one of said two surfaces an olefinic polyester of diethylene glycol and a dicarboxylic acid containing substantial portions of maleic acid, said polyester having a molecular weight less than about 5000 and being in solution in a quantity of styrene; and placing said two surfaces one against the other with the introduction therebetween of a peroxide catalyst to effect a polymerization reaction involving said polyester and said styrene at a temperature under 90° C. without evolution of any volatile material, thereby effecting strong adhesion of said two surfaces.

15. The process for making a transducer device having an electromechanically sensitive element one surface of which is secured to another similarly shaped surface comprising: applying to one of said two surfaces a polyester of a dicarboxylic acid and a glycol, at least some of whose monoester units are olefinic, which has a molecular weight less than about 5000, and which is in solution in a quantity of a polymerizable liquid aromatic compound with an olefinic side chain; applying to the other of said surfaces a peroxide catalyst; and subsequently placing said two surfaces one against the other to effect a polymerization and cross-linking reaction involving said polyester and said aromatic compound at a temperature under 90° C. without evolution of any volatile material, thereby effecting strong adhesion of said two surfaces.

16. The process for making a transducer device having an electromechanically sensitive element one surface of which is secured to another similarly shaped surface comprising: applying to at least one of said two surfaces an essentially linear olefinic polyester, which is partially polymerized to enable further rapid polymerization for bonding purposes at unelevated temperatures, and

which is in a state of molecular dispersion in a quantity of a polymerizable liquid aromatic compound with an olefinic side chain to increase the liquidity of said polyester and permit a satisfactory bonding contact with elemental areas of said surfaces in spite of the substantially large average molecular size of said partially polymerized polyester; and placing said two surfaces one against the other with the introduction therebetween of a catalyst to effect a polymerization and cross-linking reaction involving simultaneously said partially polymerized polyester and said polymerizable aromatic compound at a temperature in the neighborhood of room temperature without evolution of any volatile material, thereby effecting strong adhesion of said two surfaces.

17. The process for making a transducer device having an electromechanically sensitive element one surface of which is secured to another similarly shaped surface comprising: applying to at least one of said two surfaces a bonding material, which is partially polymerized to enable further rapid polymerization for bonding purposes at temperatures not highly elevated, and which is in a state of molecular dispersion in a quantity of a polymerizable liquid solvent material to increase the liquidity of said bonding material and permit a satisfactory bonding contact with elemental areas of said surfaces in spite of the substantially large average molecular size of said partially polymerized bonding material; and placing said two surfaces one against the other with the introduction therebetween of a catalyst to effect a polymerization reaction involving simultaneously said partially polymerized bonding material and said polymerizable solvent material at a temperature under 90° C. without evolution of any volatile material, at least one of said surfaces being cut from a single crystal of a polar compound, thereby effecting strong adhesion of said last-mentioned surface and the other of said two surfaces.

18. The process for making a transducer device having an electromechanically sensitive element one surface of which is secured to another similarly shaped surface comprising: applying to at least one of said two surfaces a bonding material, which is partially polymerized to enable further rapid polymerization for bonding purposes at temperatures not highly elevated, and which is in a state of molecular dispersion in a quantity of a polymerizable liquid solvent material to increase the liquidity of said bonding material and permit a satisfactory bonding contact with elemental areas of said surfaces in spite of the substantially large average molecular size of said partially polymerized bonding material; and placing said two surfaces one against the other with the introduction therebetween of a catalyst to effect a polymerization reaction involving simultaneously said partially polymerized bonding material and said polymerizable solvent material at a temperature under 90° C. without evolution of any volatile material, both of said surfaces being surfaces of single-crystalline plates of a polar compound, thereby effecting a strong adhesion of said two plates so that piezoelectric deformations of the regions near said two surfaces in opposite senses are associated with flexural movements of the composite element.

14

ANDREW SZEGVARI.  
CHARLES K. GRAVLEY.

## References Cited in the file of this patent

## UNITED STATES PATENTS

| Number     | Name      | Date          |
|------------|-----------|---------------|
| Re. 20,213 | Sawyer    | Dec. 22, 1936 |
| 1,995,257  | Sawyer    | Mar. 19, 1935 |
| 2,453,665  | Kropa     | Nov. 9, 1948  |
| 2,453,666  | Kropa     | Nov. 9, 1948  |
| 2,472,963  | Singleton | June 14, 1949 |

## OTHER REFERENCES

Experimental Plastics and Synthetic Resins,

D'Alelio, "Low Pressure Laminating," 1946, pp. 67-8.

Industrial and Engineering Chemistry, "Polyester Styrene Resin Systems," Ebers et al., Jan. 5 1950, pp. 114-119.

Proceedings of the I.R.E., "Standards on Piezoelectric Crystals," vol. 37, Issue 12, pp. 1378-1395, Dec. 1949.

Optical Methods of Chemical Analysis, Gibb, 10 "The Nichol Prism," pages 256-7, 1942.